

1

2,926,081

## PROCESS OF SMELTING ZINC CONTAINING LEAD ORES

Werner Schwartz, Frankfurt am Main, Eschersheim, Germany, assignor to Dravo Corporation, Pittsburgh, Pa., a corporation of Pennsylvania

No Drawing. Application May 15, 1956  
Serial No. 584,881

8 Claims. (Cl. 75—77)

This invention relates to the process of extracting lead from lead ores containing zinc and is for a method of direct separation of the lead and the zinc from the ore.

Lead is generally obtained from naturally occurring sulphide ore. In cases where the ore or ore concentrate is quite pure, it is smelted by the well-known "roast-reaction" process. This involves the conversion of the lead sulphide (PbS) with lead compounds containing oxygen, such as lead oxide (PbO) and lead sulphate (PbSO<sub>4</sub>). These oxygen bearing compounds may be transiently produced in the smelting process, and it is also well-known to roast or sinter the sulphide ore in the presence of oxygen to produce the oxygen containing compounds mentioned above. The roast reaction may be expressed as follows:



and can be further reduced to the simple formula:



It can be carried out simply by blowing an air stream into the heated ore whereby at approximately 1000° C. the above reaction takes place and the molten lead flows down and gathers in a pool covered by a layer of slag that protects the lead from oxidation.

This procedure is simple; the reaction is exothermic and little or no fuel is required and no addition materials need be used. However it can be used advantageously only with lead sulphide ore of high purity, that is ore which is not only relatively free of gangue, but which does not contain zinc. Such ore, however, is becoming increasingly unavailable, since zinc in the form of zinc sulphide is present in appreciable amounts in most ore presently being produced.

Zinc sulphide, or zinc oxide produced therefrom in the roast-reaction process combines with the slag, greatly increasing its viscosity and increasing the smelting temperature of the slag to a point where the roast-reaction procedures above described are retarded.

Therefore, the roast-reaction process can not be used with lead ores containing zinc. Instead, the smelting must be effected in a "roast-reduction" process in which the lead and zinc sulphides are first completely oxidized and the oxide then reduced in a shaft furnace with a high grade coke used as a reducing agent.

The present invention is based on the discovery that the roast-reduction of lead sulphide ore concentrates containing substantial amounts of zinc can be effected by the following procedure:

(1) The charge is prepared from a mixture containing the sulphide ore and more chemically combined oxygen than is required to satisfy reaction number 3 above, and in addition convert the zinc sulphide to zinc oxide. The combined oxygen can be accomplished by sintering ore concentrate on a sintering band in a known manner to partially or completely convert the sulphide to oxide and sulphate.

2

(2) Introducing into the charge a reducing agent such as coal or iron scrap. This will combine with any excess oxygen that may be present over and above that required to oxidize the zinc.

5 (3) Introducing into the charge a reagent which is more basic than zinc oxide and which has a higher degree of affinity for the slag than zinc oxide, so that the zinc oxide, instead of reacting with slag, will either be carried off with the furnace gases or reduced by the reducing agent and be carried off as a metallic vapor.

Instead of requiring a shaft furnace with expensive high-grade coke which often times is not available, I may use a reverberating furnace operated with oil, gas or coal as a smelter. Preferably a short rotating reverberatory furnace with a deep bath is employed. By a short furnace I mean one having a diameter greater than or at least not much less than its length. Such a furnace is used because of its economy and certain other factors that make it highly adaptable for this purpose.

15 20 Conventional equipment may be used with my process. Roasted and raw ore concentrates may be formed in the usual way, and a mix prepared that can be sintered on a Dwight-Lloyd type of downdraft sintering apparatus. A smelting furnace of known construction, preferably 25 as above described, may be used, and finally a dust filter is required for separating the zinc oxide from the smelter gases.

The reducing agent may be carboniferous, as anthracite or coke, or it may be ferrous, as scrap iron, steel or the 30 like. The basic addition for the slag is preferably sodium carbonate (calcined) but other materials of an equivalent character are lime-glass, potash, borax, sodium sulphate and like alkaline materials, or materials for which the slag impurities have a greater affinity than 35 they do for zinc oxide.

In the practice of the invention, lead ore concentrate containing zinc is roasted to a desired extent. This is conveniently accomplished on a downdraft sintering apparatus, in which case raw concentrate is mixed with 40 sinter from a previous run in order to have a mix that is physically adaptable for sintering. The resulting sinter is crushed or granulated to a convenient small mesh size. Unroasted ore concentrate in a finely divided state is introduced with water and the crushed sinter into a 45 mixer, the amount of water being sufficient to cause the unroasted material to coat the coarser roasted grains. The particles thus produced by agitating or churning the material in the mixer comprise a core which has already been sinter-roasted surrounded by a layer of non-sintered 50 ore concentrate.

The prepared material is then charged into a short drum smelting furnace along with the calcined sodium carbonate or other basic reagent, and with the reducing agent, which may be broken coal, iron scrap, steel chips 55 or the like, and the charge smelted in the usual way. After the charge has been smelted for about one-third the normal time, the accumulated lead, generally amounting to about 40–60% of the total lead content, may be drawn off. It will be of a high degree of purity, around 99.9% 60 pure. Thereafter the smelting operation can be continued until the charge has been completely smelted, and the additional lead drawn off. This metal will be of normal commercial purity but of a less pure quality than that first removed. A short drum furnace adapts itself 65 well to this procedure.

During the smelting, the gases from the short drum or other smelting furnace are directed through a dust filter or collector. The zinc, instead of being combined in the slag, is recovered by such dust filter or collector as zinc 70 oxide.

As a typical example, 1000 kg. of roasted and sintered lead concentrate was mixed with a like amount of non-

sintered ore concentrate. The sintered concentrate showed an analysis of 70.6% lead and 4.8% zinc. The non-sintered concentrate showed 70.2% of lead and 5.1% of zinc. From this mixture 100 grams were tested by being subjected to a temperature of 1250° C. in a fire clay crucible. The resulting material had a lead content of 85%, and there was a slag of yellow color, indicating the presence of lead oxide. This is a quick test to show that more combined oxygen was present than that stoichiometrically required.

Of the mixture 67 kg. were then introduced into a short drum smelting furnace together with 6.7 kg. of calcined soda ash and 4.0 kg. of finely divided anthracite. The soda so added ranges between 5% and 20% of the ore charge, about 10% being indicated as preferable. The reducing agent should be in an amount to assure that the flue gases are non-oxidizing, that is, that all surplus oxygen is reacted. After two hours of firing at a temperature of about 1250° C., 45.7 kg. of metal were tapped out of the furnace, and this was of about 99.5% purity. There were 6.5 kg. of slag containing about 12.5% of zinc. Also 3.05 kg. of flue dust were collected, and analysis proved this to contain 70% of zinc oxide.

The foregoing example shows that 67% of the total zinc was recovered in the flue dust, principally as zinc oxide. At the same time 96% of the total lead was recovered. When operating with concentrates containing higher amounts of zinc than above given, more zinc can be extracted. For example, when an ore concentrate having 8% of zinc and 63.7% of lead was processed in this way, 78% of the total zinc was obtained in the flue dust.

From the foregoing, it is to be seen that the roast-reaction of the lead proceeded normally; the zinc was oxidized and the zinc oxide, which is chemically basic, was prevented from reacting with acid slag and impurities by the use of the more alkaline reagent, such as soda. A surplus of oxygen in combined form over the theoretically exact amount assures adequate oxygen to effect the process while reducing agent binds the surplus in a manner harmless to the desired result.

While a specific method of preparing the charge has been described, various changes and modifications may be used in the procedure to accomplish the process.

What is claimed is:

1. A process of smelting lead ore containing zinc which comprises initially preparing a charge of roasted and unroasted ore concentrate in a proportion to provide in the mix chemically bound oxygen in excess of the theoretical requirement of the roast-reaction process of the lead content plus there being at least sufficient additional chemically bound oxygen to oxidize the zinc to zinc oxide, initially mixing a reducing agent with this charge, then smelting the charge so prepared under conditions conducive to the removal of the zinc as zinc oxide vapor.

2. A process of smelting lead ore containing zinc which comprises preparing a charge of roasted and unroasted ore concentrates in a proportion to provide combined oxygen over and above the amount theoretically required to effect the roast-reaction of the lead and also oxidize the zinc, introducing a reducing agent into the charge before smelting, smelting the charge, and maintaining the slag and impurities sufficiently alkaline that zinc oxide produced in the smelting is carried out with the smelter gases.

3. The method of smelting lead ore containing zinc as defined in claim 1, wherein an alkaline substance more reactive with slag and slag impurities than zinc oxide is introduced into the charge to retard reaction of the zinc oxide with the slag.

4. The method of smelting lead ore containing zinc as defined in claim 1 wherein the charge is prepared by first agitating roasted sintered ore concentrate in granular form with finely divided unroasted ore concentrate and water to coat the sintered granules with the unroasted ore.

5. The process of smelting lead ore containing zinc as defined in claim 2 in which the roasted ore in the form of sintered granules and the non-sintered ore concentrate is coated on such granules.

6. A process for smelting lead ore containing zinc which comprises roasting zinc-containing lead sulphide ore concentrates to produce mixed lead oxide and lead sulphate, then mixing therewith additional similar lead ore concentrates in the form of lead sulphide in amounts such that the combined oxygen is present in the mix in an amount greater than that required for the stoichiometric roast-reaction of sulphur and oxygen, adding to said mixture soda and a reducing agent from the group consisting of carbon and iron before smelting, the soda being in an amount sufficient to maintain a slag in the smelting furnace that is essentially basic, smelting the charge so prepared and recovering the lead from the smelting operation in metallic form and the zinc as zinc oxide in flue dust from the smelter.

7. A process for smelting lead ore containing zinc as defined in claim 6 wherein the content of combined oxygen in the furnace charge is adjusted in such manner that substantially the total amount of zinc present in the ore is oxidized to zinc oxide and the following complete roast-reaction effected:



8. The process of reducing lead sulfide ore concentrate containing zinc which comprises preparing a mixture of ore which is partially roasted to convert the sulfide to lead oxide and lead sulfate while the remainder of the mix is unconverted ore and in which the proportion of combined oxygen is more than sufficient to satisfy the roast-reaction expressed as  $\text{PbS} + \text{O}_2 = \text{Pb} + \text{SO}_2$  and convert the zinc sulfide to zinc oxide, adding to the mix so prepared and before smelting a reducing agent then smelting this mixture to reduce the lead ore to metal and removing the zinc with the smelter gases as zinc oxide.

#### References Cited in the file of this patent

#### UNITED STATES PATENTS

|           |                  |               |
|-----------|------------------|---------------|
| 481,500   | Lewis            | Aug. 23, 1892 |
| 543,753   | Roux             | July 30, 1895 |
| 681,609   | Bechi            | Aug. 27, 1901 |
| 1,744,174 | Oldright         | Jan. 21, 1930 |
| 1,804,054 | Hayward          | May 5, 1931   |
| 2,006,257 | Betterton        | June 25, 1936 |
| 2,416,628 | Kalling et al.   | Feb. 25, 1947 |
| 2,461,280 | Isbell           | Feb. 8, 1949  |
| 2,797,158 | Wendeborn et al. | June 25, 1957 |

UNITED STATES PATENT OFFICE  
CERTIFICATE OF CORRECTION

Patent No. 2,926,081

February 23, 1960

Werner Schwartz

It is hereby certified that error appears in the printed specification of the above numbered patent requiring correction and that the said Letters Patent should read as corrected below.

Column 1, line 62, for "roast-reduction" read -- roast-reaction --; column 3, line 22, for "12,5%" read -- 12.5% --.

Signed and sealed this 20th day of September 1960.

(SEAL)

Attest:

KARL H. AXLINE

Attesting Officer

ROBERT C. WATSON  
Commissioner of Patents